# EUROPEAN PATENT SPECIFICATION

(11) **EP 1 027 988 B1**
(45) Date of publication and mention of the grant of the patent: **11.04.2007**
(21) Application number: 99906481.9
(22) Date of filing: 25.02.1999
(51) Int. Cl.: B41J 2/045, B41J 2/05, B41J 2/14, B41J 2/16

(54) **HYDROPHILIC STRUCTURE**
HYDROPHILE STRUKTUR
STRUCTURE HYDROPHILE

(30) Priority: 27.08.1998 JP 24235598
(43) Date of publication of application: 16.08.2000
(73) Proprietor: SEIKO EPSON CORPORATION, Shinjuku-ku Tokyo 163-0811 (JP)
(72) Inventor: KARASAWA, Yasushi, Seiko Epson Corporation, Suwa-shi, Nagano 392-8502 (JP); ATOBE, Mitsuro, Seiko Epson Corporation, Suwa-shi, Nagano 392-8502 (JP)
(74) Representative: Hoffmann, Eckart
(86) International application number: PCT/JP1999/000870
(87) International publication number: WO 2000/012313

(56) References cited:
- JP-A- 5 312 153
- JP-A- 8 267 646
- JP-A- 8 318 628
- JP-A- 9 278 431
- JP-A- 9 331 653
- JP-A- 10 157 141
- JP-A- 59 004 897
- PATENT ABSTRACTS OF JAPAN vol. 1997, no. 09, 30 September 1997 (1997-09-30) & JP 09 127302 A (SEIKO EPSON CORP), 16 May 1997 (1997-05-16)
- PATENT ABSTRACTS OF JAPAN vol. 013, no. 369 (M-860), 16 August 1989 (1989-08-16) & JP 01 123752 A (NEC CORP), 16 May 1989 (1989-05-16)
- PATENT ABSTRACTS OF JAPAN vol. 018, no. 576 (M-1697), 4 November 1994 (1994-11-04) & JP 06 210859 A (CANON INC), 2 August 1994 (1994-08-02)
- PATENT ABSTRACTS OF JAPAN vol. 1996, no. 07, 31 July 1996 (1996-07-31) & JP 08 058096 A (CANON INC), 5 March 1996 (1996-03-05)
- PATENT ABSTRACTS OF JAPAN vol. 1997, no. 01, 31 January 1997 (1997-01-31) & JP 08 230185 A (BROTHER IND LTD), 10 September 1996 (1996-09-10)

## Description

### TECHNICAL FIELD

The present invention relates to a hydrophilic structure superior in hydrophilicity, an ink-jet recording head having an ink-jet surface superior in hydrophilicity, methods for manufacturing such a hydrophilic structure and such an ink-jet recording head, an ink-jet recording apparatus, and structural members for a micro-pump, frosted glass, a bearing, a bath tub, a bathroom tile, a wash stand, a pipe for a heat exchanger, a blood circuit for an artificial lung, etc.

### BACKGROUND ART

In the background art, there have been devised various hydrophilic treatment methods for the purpose of preventing fogging of window glass or the like in a building, a car or the like, for the purpose of preventing fouling of a solid surface, or for other purposes. Of these hydrophilic treatment methods, JP-B-61-83106 and Japanese Patent No. 2756474 disclose a hydrophilic treatment method using optically semiconducting metal oxide. In this hydrophilic treatment method, optically semiconducting metal oxide such as titanium oxide or the like is formed on a solid surface, and this solid surface is irradiated with light in an ultra-violet region so that hydrophilicity is developed on the solid surface.

Incidentally, in an ink-jet recording head, glass, metal or the like is used for the constituent material of an ink-jet surface (except ink-jet holes). Therefore, when there appears a portion to which it is difficult for ink droplets to adhere, for example, due to the adhesion of fat or oil from the environment, there is a fear that the linearity of ink droplets to be discharged is lost so that troubles such as printing instability or the like may hinder good recording. Thus, it is requested that either a hydrophilic state easy to get wet with ink or a water repellent state difficult to get wet with ink can be kept for a long term in the ink-jet surface of the ink-jet recording head.

However, the above-mentioned background-art hydrophilic treatment method using optically semiconducting metal oxide does not have such a function satisfactorily. Particularly, when the hydrophilic treatment method is applied to an ink-jet recording head, it has a problem as follows.

That is, the hydrophilic treatment method using optically semiconducting metal oxide required irradiating the optically semiconducting metal oxide with light including an ultra-violet component, but the structure of an ink-jet recording head was so complicated that its ink-jet surface could not be always irradiated with light including an ultra-violet component. As a result, any good hydrophilic state could not be obtained in a portion which was not irradiated with the light. Even if a hydrophilic state could be obtained temporarily, the hydrophilic state could not be kept over a long period of time.

PCT/WO96/29375 also proposes a method in which a surface of a mirror lens, window glass, goggles, a bath tub, or other articles is coated with a photocatalyst semiconductor material and then irradiated with light so as to obtain hydrophilicity, anti-fogging properties, and easiness in cleansing by rinsing. Even in this method, however, irradiation with light having a comparatively short wavelength is necessary so that any good hydrophilic state cannot be obtained in a portion which is not irradiated with the light. In addition, since there is a problem in durability, even if a hydrophilic state can be obtained temporarily, the hydrophilic state cannot be kept over a long period of time.

Further, JP-A-5-312153 proposes a method in which the surface of a channel of a micro-pump is subject to graft treatment for the purpose of preventing generation of bubbles in the channel and improving the constant flow rate property. Even in this method, however, there is a possibility that any hydrophilic state cannot be kept over a long period of time because there is a problem in durability.

JP-A-1-250265 also proposes a method in which a blood circuit of an artificial lung is coated with HEMA or the like in order to improve its wettability with blood and its gas exchangeability. Also in this method, however, there is a problem in adhesive properties of the coating polymer, and there is a disadvantage in durability.

JP-A-06 210 859 discloses an inkjet head and the particular structure of its nozzle surface. A water repelling region is provided closely to the nozzle openings and a hydrophilic area is provided in a belt-like manner at a predetermined distance from the nozzle openings. The hydrophilic region comprises groove-like areas on both sides of the nozzle openings the grooves extending in parallel to a nozzle row. An outer hydrophilic portion has a plurality of island-like hydrophilic regions provided on the side of the grooves remote from the nozzles. No details are provided with respect to the island-like hydrophilic regions in this document.

### DISCLOSURE OF THE INVENTION

It is an object of the present invention to provide a hydrophilic structure which can keep hydrophilicity for a long term.
(1) According to an aspect of the present invention, there is provided a hydrophilic structure according to claim 1.
(2) Embodiments of the present invention are described in claims 2 to 4.

The hydrophilic structure according to the present invention has a structure in which an artificial irregular shape is provided on a base to thereby obtain not only a stable super hydrophilic function but also high durability and high mar-proof property.

According to the present invention, not only a super hydrophilic function but also high durability and high mar-proof property are obtained by the above-mentioned hydrophilic structure. The details of the present invention including its operation principle will be explained in Embodiment 1 which will be described below. Further, according to the present invention, it is defined that the conception of super hydrophilic includes super lipophilic.

### BRIEF DESCRIPTION OF THE DRAWINGS

Fig. 1 is an explanatory view of a structure according to Embodiment 1 of the present invention;
Fig. 2 is a view for explaining the dimensions of a recess portion and a protrusion portion in Fig. 1;
Fig. 3 shows different plan views of the structure 100 in Fig. 1;
Fig. 4 is an exploded perspective view of an ink-jet recording head according to Embodiment 2 of the present invention;
Fig. 5 is a series of sectional views showing a manufacturing process for forming a structure on the surface of a second plate in Embodiment 2;
Fig. 6 is a top view of the second plate on which the structure is formed;
Fig. 7 is a series of sectional views showing a manufacturing process for a second plate in a Comparative Example;
Fig. 8 is a series of sectional views showing a manufacturing process for forming a structure on the surface of a second plate in Embodiment 3 of the present invention;
Fig. 9 is a series of sectional views showing a manufacturing process for forming a structure on the surface of a second plate in Embodiment 4 of the present invention;
Fig. 10 is a series of sectional views showing a manufacturing process for forming a structure on the surface of a second plate in Embodiment 5 of the present invention;
Fig. 11 is a series of sectional views showing a manufacturing process for forming a structure on the surface of a second plate in Embodiment 6 of the present invention;
Fig. 12 is an explanatory view showing an example of a mechanism near an ink-jet head manufactured through any one of the manufacturing processes of Embodiments 2 to 6;
Fig. 13 is an external appearance view of an ink-jet recording apparatus on which the mechanism of Fig. 12 is mounted;
Fig 14 is a sectional view of a micro-pump according to Embodiment 9 of the present invention;
Fig. 15 depicts explanatory views showing a mechanism for manufacturing a tube in Fig. 14;
Fig. 16 shows sectional views of different frosted glass according to Embodiment 10 of the present invention;
Fig. 17 is a sectional view of a mechanism for a watch according to Embodiment 11 of the present invention; and
Fig. 18 shows perspective views of a bathroom and a wash stand according to Embodiment 12 of the present invention.

### THE BEST MODE FOR CARRYING OUT THE INVENTION

### Embodiment 1.

Fig. 1 is an explanatory view of a hydrophilic structure according to Embodiment 1 of the present invention. In Fig. 1, in a hydrophilic structure 100, recess portions 17 and protrusion portions 18 are formed on the surface of a silicon substrate 11, and a hydrophilic film 20 is formed on the surfaces of the recess portions 17 and the protrusion portions 18. In this structure, in addition to the performance of the hydrophilic film 20, fluid 21 permeates into the recess portions 17 by capillarity so that the hydrophilicity of the surface of the structure is improved. Therefore, these irregularities are adjusted to dimensions such that the fluid 21 can enter the recess portions 17 easily by capillarity. After formation of the irregularities, the hydrophilic film 20 may be formed, for example, by graft polymerizing, silica coupling, silicon oxidizing, or the like. In this embodiment, since the silicon substrate 11 is used as the base, the hydrophilic film 20 is formed by silicon oxidizing. Although this embodiment shows the case where the hydrophilic film 20 is formed, a base having a hydrophilic function, for example, glass, or the like, may be used with irregularities formed thereon.

Fig. 2 is a view for explaining the dimensions of each recess portion 17 and each protrusion portion 18 in Fig. 1. In Fig. 2, the symbol A designates a protrusion width (depending on the mask design); B, a groove width (depending on the mask design); C, a working quantity (depending on the depth and etching time); and D, a side wall angle (depending on the etching conditions).

In the case of an ink-jet recording apparatus for jetting ink droplets each having a diameter of tens of µm, the above-mentioned widths A and B are restricted by themselves in order to obtain stable hydrophilic performance near nozzle holes. In addition, the above-mentioned quantity C needs to have a certain degree of depth enough to diffuse permeating ink droplets in the recess portion stably. Therefore, the above-mentioned widths A and B are restricted in a range of from 0.2 to 500 µm, preferably from 0.5 to 30 µm, more preferably from 1 to 10 µm. In addition, the above-mentioned quantity C is restricted to a depth of 1 µm or more, preferably 3 µm or more, more preferably 5 µm or more. The evenness of the height of the protrusion portions is restricted within 0.5 times as large as the value of the widths A and B, preferably within 0.3 times, more preferably within 0.1 times, from the point of view of the mar-proof property.

Fig. 3 is a plan view of the hydrophilic structure 100 in Fig. 1. Fig. 3(A) shows an example in which the protrusion portions 18 are distributed regularly. Fig. 3(B) shows an example in which the protrusion portions 18 are arranged in the form of lines. Fig. 3(C) shows an example in which the protrusion portions 18 are arranged in the form of a lattice. Although Fig. 3(A) shows an example in which the protrusion portions 18 are square prisms, they may be various pillars such as triangular prisms, pentagonal prisms, hexagonal prisms, circular columns, etc., or cones.

### Embodiment 2.

Fig. 4 is an exploded perspective view of an ink-jet recording head according to Embodiment 2 of the present invention. As illustrated, the ink-jet recording head has a configuration in which a first plate 1 and a second plate 2 are laminated on each other so that an ink supply portion 3, pressure chambers 4 for jetting ink, and channels 5 for passing the ink therethrough are formed. The pressure chambers 4 jet ink by using vibration of a diaphragm such as an electrostatic diaphragm vibrated by static electricity, a piezoelectric vibrator such as an PZT, or the like, or by heating of a heating element. In the second plate 2, nozzle holes 6 are formed perpendicularly to the channels 5. The hydrophilic structure 100 in Fig. 1 is formed on the surface of the second plate 2, and the hydrophilic film 20 is formed on the surface of the hydrophilic structure 100.

Fig. 5 is a sectional view showing a manufacturing process for forming the hydrophilic structure on the surface of the second plate 2. Fig. 6 is a top view of the second plate 2 in which the hydrophilic structure has been formed on the surface. Here, description will be made about the case where the surface of a silicon substrate is worked by a photolithography method and a trench dry etching method so that a hydrophilic structure is formed.
① First, a 4-inch single-crystal silicon wafer of the (100) crystal orientation is prepared as the base of the second plate 2. As shown in Fig. 5(a), a silicon oxide film 12 having a thickness of about 1,000 Angstroms is formed on at least one surface of the single-crystal silicon substrate 11 by use of a thermal oxidation method.
② Next, as shown in Fig. 5(b), about 2 ml of photosensitive resin OFPR-800 (viscosity; 30 cps) made by TOKYO OHKA KOGYO CO., LTD. is dropped onto the thermally oxidized silicon film 12 of the single-crystal silicon substrate 11, and spin-coated for 30 seconds at the velocity of 5,000 rotations per minute, so that a photosensitive resin layer 13 is formed. By these spin-coat conditions, the photosensitive resin can be applied so that the average film thickness is about 1 µm, and the variation in the wafer surface is 10%. Then, the coating film thickness is changed desirably in accordance with the dimensions of a groove to be worked, or the like. The maximum value of the thickness of the photosensitive material film to be applied is 2 µm when the dimension of one side of the groove is 2µm.
③ Next, the substrate 11 is dried for 30 minutes in an oven at a temperature of 90°C, and cooled down to the room temperature. As shown in Fig. 5(c), protrusion-portion-expected areas 13 each of which is 0.2µm to 200µm square are photolitho-patterned in the substrate 11. Then, the photosensitive resin is solidified by the oven at a temperature of 120°C, so that the etching-proof property is improved.
④ As shown in Fig. 5(d), the silicon oxide film in groove-expected areas is etched with fluoric acid, and the photosensitive resin is removed in a stripping solution.
⑤ Next, by use of a trench dry etching apparatus, a plasma synthetic film 14 is formed with gas containing C and F, as shown in Fig. 5(e). Succeedingly, after the dry etching apparatus has been evacuated, silicon in the area of a silicon substrate bottom 15 is etched with plasma of gas of the chemical formula SF6 or CF4, as shown in Fig. 5(f). Then, as shown in Fig. 5(f), the silicon oxide film 12 exists in portions which shall be protrusion portions, so that the portions are not etched. On the other hand, portions which shall be recess portions are anisotropically etched effectively by the effect of the plasma synthetic film formed on portions which shall be side walls of the protrusion portions. Such a plasma synthesis step and such a plasma etching step are repeated. As a result, grooves each having a depth of about 5µm are etched in the surface of the single-crystal silicon substrate 11 so that the recess portions 17 and the protrusion portions 18 are formed, as shown in Fig. 5(g). These protrusion portions 18 are laid out regularly on the surface of the single-crystal silicon substrate 11, as shown in Fig. 3.
⑥ Next, nozzle holes 6 (see Fig. 4) are worked, and a silicon oxide film is formed on the single-crystal silicon substrate 11 by a thermal oxidation method (alternatively, a sputtering method or a sol-gel method may be used) so as to obtain a hydrophilic film 20 (Fig. 5(h)).
⑦ Finally, a first plate 1 is bonded with the second plate 2 formed thus so that an ink-jet recording head is completed.

### (Example 1)

As Example 1 of the present invention, examples shown in Table 1 were attempted in the above-mentioned Embodiment 2. First, base materials of samples 1 to 7 were prepared for the substrate 11 of the second plate. Then, the protrusion-portion-expected areas 13 (see Fig. 5(c)) were formed by patterning squares each in a range of from 0.2 µm to 1,000 µm. In addition, the hydrophilic film to be formed on the second plate 2 was formed by depositing silicon oxide.

This hydrophilic treatment was not performed on the samples 2, 4 and 6. [Table 1]

| Number | Base | Protrusion size (micron square) | Hydrophilic treatment |
|---|---|---|---|
| Sample 1 | Single-crystal silicon | 0.2 | Yes |
| Sample 2 | Single-crystal silicon | 0.2 | No |
| Sample 3 | Glass | 5 | Yes |
| Sample 4 | Single-crystal silicon | 5 | No |
| Sample 5 | Quartz | 10 | Yes |
| Sample 6 | Single-crystal silicon | 10 | No |
| Sample 7 | Quartz | 500 | Yes |
| Sample 8 | Glass | 500 | No |

### (Comparative Example)

Fig. 7 is a sectional view showing a manufacturing process as a Comparative Example in which hydrophilic treatment is applied to a second plate of stainless steel in an ink-jet recording head configured in the same manner as in Embodiment 2. The ink-jet recording head in this Comparative Example has the same configuration as that shown in Fig. 4.
① First, a base 31 for the second plate was worked so that nozzle holes 32 were formed. Then, the base 31 was subjected to ultrasonic cleaning with an alkali detergent, as shown in Fig. 7(a).
② Next, as shown in Fig. 7(b), titanium oxide 33 was deposited on the second plate base 31.
③ Finally, a first plate 1 was bonded with the second plate 2 formed thus so that an ink-jet recording head was completed.

Table 2 shows contact angles of the second plates against ink and water in this Example and Comparative Example. Further, data of Comparative Example were obtained immediately after irradiation with ultra-violet rays.

**[Table 2]**

| Number | | Water contact angle (degrees) | Ink contact angle (degrees) |
|---|---|---|---|
| Example | Sample 1 | 6 | 2 |
| | Sample 2 | 20 | 12 |
| | Sample 3 | 4 | 2 |
| | Sample 4 | 30 | 14 |
| | Sample 5 | 4 | 4 |
| | Sample 6 | 30 | 16 |
| | Sample 7 | 20 | 10 |
| | Sample 8 | 20 | 10 |
| Comparative Example | | 10 | 4 |

Each sample, except those which used silicon not-subjected to hydrophilic treatment, was superior in hydrophilicity with the contact angle against ink not more than 10 degrees.

Each ink-jet recording head in Embodiment 1 was mounted on a recording apparatus, and subjected to a printing test in initial conditions and in accelerated conditions corresponding to 2 years in the darkness. Thus, the results were obtained as shown in Table 3. Table 3 shows the results of judgement upon printing quality, in which the mark ⊚ designates superior printing quality without ink mist adhering to the second plate surface; the mark ○, superior printing quality though ink mist adhered to the second plate surface; and the mark X, defective due to bending in flying of ink.

**[Table 3]**

| Sample number | | Printing quality | |
|---|---|---|---|
| | | Initial | After accelerated conditions corresponding to 2 years |
| Example | Sample 1 | ⊚ | ⊚ |
| | Sample 2 | ○ | ○ |
| | Sample 3 | ⊚ | ⊚ |
| | Sample 4 | ○ | ○ |
| | Sample 5 | ⊚ | ⊚ |
| | Sample 6 | ○ | ○ |
| | Sample 7 | ⊚ | ○ |
| | Sample 8 | ○ | ○ |
| Comparative Example | | ⊚ | × |

As described above, in the ink-jet recording heads in Example 1, printing quality was superior and reproducibility was also confirmed in the initial conditions and in the accelerated conditions corresponding to 2 years. Of them, the printing quality of the second plate which has protrusion portions in a range of from 0.2 µm to 500 µm and which is coated with a hydrophilic agent to thereby form a hydrophilic film aggressively was superior. However, in the Comparative Example, the hydrophilic performance was lowered and the printing quality also deteriorated due to the environment where light could not reach.

### (Example 2)

In Example 2 of the present invention, examination was made about the contact angles between water/ink and the protrusion shapes of hydrophilic structures which were arranged in tetragonal prisms, in lines and in the form of a lattice (see Figs. 3(A), (B) and (C)). Table 4 shows data of those angles. It is understood that each of the hydrophilic structures according to the present invention had a contact angle of ink of 10 degrees or less so as to obtain superior hydrophilic performance without irradiation with ultra-violet rays.

**[Table 4]**

| No | Structure dimensions | | | | | Contact angle | |
|---|---|---|---|---|---|---|---|
| | Structure | Protrusion width | Groove width | Working quantity | Side wall angle | Pure water | Ink |
| | | A (µm) | B (µm) | C (µm) | D (° ) | (° ) | (° ) |
| 1 | Square columns | 0.2 | 2.4 | 3.2 | 14 | 6 | 2 |
| 2 | Square columns | 1.0 | 6.0 | 6.8 | 1 | 10 | 4 |
| 3 | Square columns | 4.0 | 6.0 | 8.6 | 0 | 12 | 6 |
| 4 | Lines | 1.2 | 2.0 | 7.8 | 1 | 10 | 4 |
| 5 | Lines | 4.0 | 6.0 | 8.0 | 4 | 12 | 4 |
| 6 | Lattice | 4.3 | 6.0 | 10.0 | 2 | 10 | 8 |
| 7 | Lattice | 10.0 | 6.0 | 1.2 | 14 | 8 | 6 |

### (Example 3)

By use of resin as the raw material, molding was performed with the structure of Example 1 or 2 as a mold. The surface of a molded product obtained thus had a pattern of irregularities which was transferred from the surface of the mold. It was confirmed that such a structure subjected to hydrophilic treatment also had superior properties similar to those in Examples 1 and 2.

### Embodiment 3.

Fig. 8 is a sectional view showing a process for manufacturing an ink-jet recording head according to Embodiment 3 of the present invention. Fig. 8 shows a manufacturing process for forming a hydrophilic structure on the surface of a second plate 2. Here, description will be made about the case where the surface of a silicon substrate is worked by a photolithography method and an anodic electrolysis method so that a hydrophilic structure is formed.
① First, for example, a 200µm thick n-type single-crystal silicon substrate 11 of (100) plane orientation is prepared as the base of a second plate.
② Silicon nitride films 23 and 24 of 0.3µm thick are formed as etching-proof coatings on this silicon substrate 11 by a CVD apparatus, as shown in Fig. 8(a).
③ Next, after the silicon nitride film 24 is removed by a dry etching method, photolitho-etching is given to the silicon nitride film 23 so that the silicon nitride film 23 is etched in portions 22 corresponding to the recess portions 17 of the structure, as shown in Fig. 8(b).
④ Next, etching pyramids 25 shaped into V-grooves are worked in the silicon substrate 11 by an anisotropic etching method using an aqueous solution of potassium hydrate with the silicon nitride film 23 as a mask. An indium-tin oxide film (ITO film) 26 is formed on the surface of the silicon substrate 11 opposite to the surface where the silicon nitride film 23 has been formed, as shown in Fig. 8(c).
⑤ Succeedingly, an electrolytic cell is assembled so that the above-mentioned surface where the silicon nitride film 23 has been formed is in contact with electrolyte. While the silicon substrate 11 is irradiated with light at its surface opposite to the surface where the silicon nitride film 23 has been formed, grooves 27 of about 5µm deep are etched as shown in Fig. 8(d), so that the recess portions 17 and the protrusion portions 18 are produced (Fig. 8(e)).
⑥ Nozzle holes 6 (see Fig. 4) are worked, and a silicon oxide film is deposited as the hydrophilic film 20 on the second plate 2 by a vacuum deposition method (Fig. 8(f)).
⑦ Finally, a first plate 1 is bonded with the second plate 2 formed thus so that an ink-jet recording head is completed.

### Embodiment 4.

Fig. 9 is a sectional view showing a process for manufacturing an ink-jet recording head according to Embodiment 4 of the present invention. Fig. 9 shows a manufacturing process for forming a hydrophilic structure on the surface of a second plate 2. Here, description will be made about the case where the surface of a silicon substrate is worked by a photolithography method and an anisotropic wet etching method so that a hydrophilic structure is formed.
① First, a 4-inch single-crystal silicon wafer of the (100) crystal orientation is prepared as the base of the second plate 2. A silicon oxide film 112 having a thickness of about 1,000 Angstroms is formed on at least one surface of a single-crystal silicon substrate 111 by use of a thermal oxidation method, as shown in Fig. 9(a).
② Next, as shown in Fig. 9(b), about 2 ml of photosensitive resin OFPR-800 (viscosity: 30 cps) made by TOKYO OHKA KOGYO CO., LTD. is dropped onto the thermally oxidized silicon film 112 of the single-crystal silicon substrate 111, and spin-coated for 30 seconds at the velocity of 5,000 revolutions per minute, so that a photosensitive resin layer 113 is formed. By these spin-coat conditions, the photosensitive resin can be applied so that the average film thickness is about 1µm, and the variation in the wafer surface is 10%. Then, the coating thickness is changed desirably in accordance with the dimensions of a groove to be worked, or the like. The maximum value of the thickness of the photosensitive material film to be applied is 2µm when the dimension of one side of the groove is 2 µm.
③ Next, the substrate 111 is dried for 30 minutes in an oven at a temperature of 90°C, and cooled down to the room temperature. As shown in Fig. 9(c), protrusion-portion-expected areas 113, each 0.2µm to 200µm square, are photolitho-patterned so as to be left on the substrate 111. Then, the photosensitive resin is solidified by the oven at a temperature of 120°C, so that the etching-proof property is improved.
④ As shown in Fig. 9(d), the silicon oxide film in groove-expected areas is etched with fluoric acid, and the photosensitive resin is removed in a stripping solution.
⑤ Next, sectionally V-shaped etching pyramids 114 are formed in the silicon substrate 111 by an anisotropic etching method using an aqueous solution of potassium hydrate with the silicon oxide film 112 as a mask, as shown in Fig. 9(e). Then, the silicon oxide film 112 is removed (Fig. 9(f)). The etching pyramids 114 formed thus correspond to the recess portions 17 in Fig. 1. Producing the recess portions 17 results in producing the protrusion portions 18 inevitably, so that the protrusion portions 18 are laid out regularly on the surface of the single crystal silicon substrate 111, as shown in Fig. 6.
⑥ Next, nozzle holes 6 (see Fig. 4) are worked, and a silicon oxide film is deposited as the hydrophilic film 20 on the single-crystal silicon substrate 111 by a vacuum deposition method (Fig. 9(g)).
⑦ Last, a first plate 1 is bonded with the second plate 2 formed thus so that an ink-jet recording head is completed.

### Embodiment 5.

Fig. 10 is a sectional view showing a process for manufacturing an ink-jet recording head according to Embodiment 5 of the present invention. Fig. 10 shows a manufacturing process for forming a porous structure on the surface of a second plate 2. Here, description will be made about the case where the surface of a silicon substrate is worked by a photolithography method and an isotropic wet etching method so that a porous structure is formed.
① First, for example, a 200µm thick glass substrate 211 is prepared as the base of the second plate 2.
② Next, as shown in Fig. 10(b), a silicon nitride film 212 of 0.3 µm thick is formed as an etching-proof coating on this glass substrate 211 by a sputtering apparatus.
③ Next, photolitho-etching is given to the silicon nitride film 212 so that the silicon nitride film is etched in portions corresponding to the recess portions 17 of the structure, as shown in Fig. 10(b).
④ Next, as shown in Fig. 10(c), etching recess portions 215 are worked in the glass substrate 211 by an isotropic etching method using an aqueous solution of hydrofluoric acid with the silicon nitride film 212 as a mask.
⑤ Next, as shown in Fig. 10(d), the silicon nitride film 212 is removed with hot phosphoric acid so that the irregularities are completed.
⑥ Next, nozzle holes 6 (see Fig. 4) are worked, and a silicon oxide film is deposited as the hydrophilic film 20 on the glass substrate 211 by a vacuum deposition method (Fig. 10(e)).
⑦ Finally, a first plate 1 is bonded with the second plate 2 formed thus so that an ink-jet recording head is completed.

### Embodiment 6.

Fig. 11 is a sectional view showing a process for manufacturing an ink-jet recording head according to Embodiment 6 of the present invention. Fig. 11 shows a manufacturing process for forming a porous structure on the surface of a second plate 2. Here, description will be made about the case where the surface of a silicon substrate is worked by a photolithography method and an isotropic dry etching method so that a porous structure is formed.
① First, for example, a 200µm thick glass substrate 311 is prepared as the base of the second plate 2.
② Next, a photosensitive resin film 312 of about 5µm thick is formed as the etching-proof coating on this glass substrate 311 by a spin-coat apparatus, as shown in Fig. 11(a).
③ Next, the photosensitive resin film 312 is etched in portions corresponding to the recess portions 17 in the structure by photolitho-etching, as shown in Fig. 11(b).
④ Next, etching recess portions 315 are worked in the glass substrate 311 by an isotropic plasma etching method using CF4 gas with the photosensitive rein film as a mask, as shown in Fig. 11(c).
⑤ Next, the photosensitive rein film 312 is removed with hot sulfuric acid so that the irregularities are completed, as shown in Fig. 11(d).
⑥ Next, nozzle holes 6 (see Fig. 4) are worked, and a silicon oxide film is deposited as the hydrophilic film 20 on the glass substrate 311 by a vacuum deposition method (Fig. 11(e)).
⑦ Finally, a first plate 1 is bonded with the second plate 2 formed thus so that an ink-jet recording head is completed.

Also in the hydrophilic structures produced in the above-mentioned Embodiments 4 to 6, it has been confirmed that the protrusion portions are even in height, and it is therefore possible to obtain a hydrophilic function, durability and mar-proof property similar to those in the above-mentioned Embodiment 2.

In the above-mentioned Embodiments 2 to 6, a hydrophilic structure is produced by a photolithography method and an etching method, and the surface of the base of the hydrophilic structure can be replaced by the tops of protrusion portions. Accordingly, the protrusion portions inevitably become even in height with high precision.

In addition, although examples using silicon or glass substrates as the material of the second plate 2 were described in the above-mentioned Embodiments 2 to 6, the material of the second plate 2 is not limited to those materials in the present invention. Similar functions can be shown even in metal material such as stainless steel or organic polymeric material.

### Embodiment 7.

Fig. 12 is an explanatory view showing an example of a mechanism near an ink-jet head manufactured through any one of the manufacturing processes of Embodiments 2 to 6. An ink-jet head 50 is attached to a carriage 51, and this carriage 51 is movably attached to guide rails 52. Then, the position of the carriage 51 is controlled in the width direction of paper 54 fed by a roller 53. This mechanism in Fig. 12 is mounted on an ink-jet recording apparatus 55 shown in Fig. 13. It has been confirmed that high-quality printing can be obtained in printing with this ink-jet recording apparatus 55. Particularly, with respect to rubbing in cleaning, it has been confirmed that a hydrophilic function is obtained by the structure of the base material of the ink-jet head so that the ink-jet head has abrasion resistance enough to be proof against long-term use.

### Embodiment 8.

Fig. 14 is a sectional view of a micro-pump according to Embodiment 8 of the present invention. In Fig. 14, when a piezoelectric element 69 is driven to vibrate a diaphragm 70, fluid sucked from an inlet 65 is discharged from an outlet 66 through a closed space 71. The hydrophilic structure according to the above-mentioned Embodiments is formed on the surface of a channel including the closed space 71. A micro-pump having an extremely constant flow rate without producing any bubble in the channel when the micro-pump was actually driven to flow pure water into the channel could be realized because the above-mentioned hydrophilic structure was formed in the micro-pump as mentioned above.

Figs. 15(A) and (B) are explanatory views showing a mechanism for manufacturing a tube 73 communicating with the inlet 65 or the outlet 66 in Fig. 14. Fig. 15(A) is a front sectional view, and Fig. 15(B) is an enlarged sectional view taken on line B-B in Fig. 15(A). In this mechanism, for example, polyvinyl chloride accommodated in a vessel 75 is discharged in the state where a die 76 on which protrusion and recess portions have been formed is passed through a discharge portion of the vessel 75, so that irregularities are formed on the inner wall of each tube 73.

### Embodiment 9.

Figs. 16(A) and (B) are sectional views of frosted glass according to Embodiment 9 of the present invention. As shown in Figs. 16(A) and (B), a hydrophilic structure 82 is formed on the surface of each frosted glass 80, 81. Accordingly, it is difficult for dirt to adhere to the surface, and even if dirt adheres to the surface, it is possible to remove the dirt easily.

### Embodiment 10.

Fig. 17 is a sectional view showing a mechanism for a watch according to Embodiment 10 of the present invention. As shown in Fig. 17, a hydrophilic structure is formed on the inner wall of each of bearing portions 85 to 90. In this case, however, this hydrophilic structure is requested to have lipophilicity as well as hydrophilicity. It is therefore necessary to perform such a hydrophilic treatment that hydrophilic and lipophilic properties can be obtained after the treatment (hydrophilic/lipophilic treatment). Since the surface of a structure subjected to such a hydrophilic/lipophilic treatment is superior in hydrophilicity and lipophilicity, lubricating oil is retained for a long term. For example, even if the watch is driven without oiling equivalently to 10 years, the watch works normally.

### Embodiment 11.

Figs. 18(A) and (B) are perspective views of a bathroom and a wash stand according to Embodiment 11 of the present invention. Hydrophilic structures 100 according to the above-mentioned Embodiments are formed on the surfaces of a bath tub 91, bathroom tiles 92 and a wash stand 93. It is therefore difficult for dirt to adhere to the surfaces, and even if dirt adheres thereto, it is possible to remove the dirt easily.

### Embodiment 12.

The hydrophilic structure according to the present invention is usable in various applications. For example, the hydrophilic structure may be formed on the inner wall of a pipe of a heat exchanger so as to improve its thermal efficiency. Also, the hydrophilic structure may be formed on the inner wall of a blood circuit of an artificial lung so as to improve its gas exchangeability or the like.

## Claims

1. A hydrophilic structure comprising:
a base (11) having a hydrophilic surface, the base (11) being selected from the group consisting of silicon, silicon oxide and glass; wherein
the hydrophilic surface includes a pattern of equally spaced protrusions (18) and recesses (17) to attract a liquid into the recesses (17) by virtue of a capillary action,
a silicon oxide film (20) completely covers the hydrophilic surface including the protrusions (18) and the recesses (17), and
the protrusions (18) and recesses (17) have a width in the range from 0.5 to 30 µm and the recesses (17) have a depth of 1 µm or more.

2. The hydrophilic structure according to Claim 1, wherein the tops of the protrusions (18) are located substantially at the same level on the hydrophilic surface.

3. The hydrophilic structure according to Claim 1 or 2, wherein the pattern of equally spaced protrusions (18) and recesses (17) forms parallel lines on the hydrophilic surface.

4. The hydrophilic structure according to Claim 1 or 2, the pattern of equally spaced protrusions (18) and recesses (17) forms a lattice structure on the hydrophilic surface.

## Patentansprüche

1. Hydrophile Struktur, aufweisend:
eine Basis (11) mit einer hydrophilen Oberfläche, wobei die Basis (11) aus der aus Silizium, Siliziumoxid und Glas bestehenden Gruppe ausgewählt ist; bei der
die hydrophile Oberfläche ein Muster von in gleichen Abständen angeordneten Erhebungen (18) und Vertiefungen (17) enthält, die eine Flüssigkeit durch Kapillarwirkung in die Vertiefungen (17) ziehen,
ein Siliziumoxidfilm (20) die hydrophile Oberfläche einschließlich der Erhebungen und der Vertiefungen (17) vollständig bedeckt, und
die Erhebungen (18) und Vertiefungen (17) eine Breite im Bereich von 0,5 µm bis 30 µm und die Vertiefungen (17) eine Tiefe von 1 µm oder mehr haben.

2. Hydrophile Struktur nach Anspruch 1, bei der sich die Spitzen der Erhebungen (18) auf der hydrophilen Oberfläche im Wesentlichen auf gleicher Höhe befinden.

3. Hydrophile Struktur nach Anspruch 1 oder 2, bei der das Muster der in gleichen Abständen angeordneten Erhebungen (18) und Vertiefungen (17) auf der hydrophilen Oberfläche parallele Linien bildet.

4. Hydrophile Struktur nach Anspruch 1 oder 2, bei der das Muster der in gleichen Abständen angeordneten Erhebungen (18) und Vertiefungen (17) auf der hydrophilen Oberfläche eine Gitterstruktur bildet.

## Revendications

1. Structure hydrophile comprenant:
une base (11) ayant une surface hydrophile, la base (11) étant choisie dans le groupe constitué du silicium, de l'oxyde de silicium et du verre ; où
la surface hydrophile comprend un motif de saillies (18) et de renfoncements (17) également espacés pour attirer un liquide dans les renfoncements (17) en vertu d'une action capillaire,
un film en oxyde de silicium (20) couvre complètement la surface hydrophile comprenant les saillies (18) et les renfoncements (17), et
les saillies (18) et les renfoncements (17) ont une largeur dans la plage de 0,5 à 30 µm et les renfoncements (17) ont une profondeur de 1 µm ou plus.

2. Structure hydrophile selon la revendication 1, où les hauts des saillies (18) sont situés sensiblement au même niveau sur la surface hydrophile.

3. Structure hydrophile selon la revendication 1 ou 2, où le motif des saillies (18) et renfoncements (17) également espacés forme des lignes parallèles sur la surface hydrophile.

4. Structure hydrophile selon la revendication 1 ou 2, où le motif des saillies (18) et renfoncements (17) également espacés forme une structure en réseau sur la surface hydrophile.
